

## UNITED STATES PATENT OFFICE

2,251,157

## DIESEL FUEL

Edwin M. Nygaard, Woodbury, N. J., assignor to  
Socony-Vacuum Oil Company, Incorporated,  
New York, N. Y., a corporation of New York

No Drawing. Application October 23, 1940,  
Serial No. 362,412

6 Claims. (CL 44—9)

This invention has to do in a general way with the operation of internal combustion engines and is more particularly concerned with improving the operation of compression ignition or Diesel engines through the use of a fuel containing a characterizing ingredient which acts to improve its ignition quality.

In engines which operate on the Diesel cycle, where the fuel is injected into compressed air in the cylinder and ignites spontaneously, it is important that the delay period between injection and ignition be short so as to promote ease of starting and smoothness of operation. Improperly delayed ignition gives rise to the phenomenon known as knocking.

One object of this invention is to improve the ignition quality of a Diesel fuel by admixing therewith a minor proportion of a novel compound or agent in sufficient proportion to decrease the ignition delay period of the fuel. The invention also contemplates a method for accelerating the ignition of a fuel in a compression ignition engine by admixing with the fuel, prior to its injection into the compressed air of the cylinder, a minor proportion of this characterizing ingredient.

This invention is predicated upon the discovery that a specific group of organic nitrogen compounds, the aromatic diazo alkyl ethers, possesses the property of decreasing the ignition delay period of Diesel fuels when admixed therewith in minor proportions.

The term aromatic diazo alkyl ether as used herein applies to compounds having the general formula  $R-N=N-O-R'$ , wherein  $R$  is selected from the group consisting of aromatic radicals and substituted aromatic radicals and  $R'$  is an alkyl group. These compounds may be prepared by various procedures described in the literature (Ber. 27, 672 (1894), Pechman and Frobenius; Ber. 36, 2505 (1903) H. Euler; Ber. 28, 227 (1895) E. Bamberger). One general procedure for preparing these compounds is by the reaction of silver diazoates with alkyl iodides. This reaction may be formulated as follows:



The silver diazoate employed in the foregoing procedure is prepared from the sodium derivative of an  $N$ -nitroso aromatic amine and silver nitrate according to the following equation:



and upon rearrangement:



As aforesaid, the term "aromatic diazo alkyl

ether" includes compounds in which the aromatic group ( $R$ ) is either unsubstituted or substituted. Because of their increased stability the aromatic group ( $R$ ) bearing a nitro substituent in the para position is preferred.

Further details in the procedure for synthesizing the compounds contemplated herein may be obtained from the following example describing the preparation of a specific compound within 10 the preferred group.

## EXAMPLE

Preparation of *p*-nitro benzene diazo methyl ether

15 A. The sodium derivative of *p*-nitrophenyl nitrosamine was first prepared according to the following procedure: Two parts of *p*-nitroaniline were added to a solution of 2.9 parts of concentrated hydrochloric acid in 12.1 parts of water. The mixture was cooled to 0° C., and to it was added a solution of 1 part sodium nitrite in 7.2 parts of water. The foregoing mixture was added quickly to a rapidly agitated NaOH solution heated to a temperature of 55–60° C. The NaOH solution consisted of 12.2 parts sodium hydroxide in 55.5 parts of water. The precipitated product was filtered and washed once with cold water and purified by recrystallization from 90 per cent ethyl alcohol heated to 60° C. It 20 may be represented by the formula:



25 B. Silver-*p*-nitrobenzene diazoate was prepared by dissolving 1.1 parts of the sodium derivative of *p*-nitrophenyl nitrosamine prepared by procedure "A" in 22.2 to 27.8 parts of water, filtering the mixture to remove a small quantity of insoluble material and slowly adding to the filtrate with agitation a solution of one part of silver nitrate in about 11.1 parts of water. The precipitated product was filtered, washed with water, and carefully dried on a porous plate. It 30 may be represented by the formula:



35 C. Para-nitro benzene diazo methyl ether was prepared by suspending 1.3 parts of the dried silver compound obtained by procedure B in 13.5 parts of dry diethyl ether and adding thereto 1.0 part of methyl iodide dissolved in about two 40 or three times its own volume of dry ether. The mixture was agitated vigorously for about 3 hours, after which the precipitated silver iodide was removed by filtration and the product recovered by evaporation of the ether filtrate under 45 vacuum at room temperature. This final product

uct, p-nitro benzene diazo methyl ether has the formula:



The corresponding ethyl derivative (p-nitro benzene diazo ethyl ether) having the formula:



was obtained in like manner using ethyl iodide in place of methyl iodide.

To demonstrate the effectiveness of the addition agents contemplated herein as improvers for Diesel fuel, the two compounds obtained according to the procedure in the foregoing examples were blended with typical Diesel fuels (indicated as "Fuel A" and "Fuel B" below), and the ignition quality of the blends was ascertained by determination of their cetane numbers. The cetane numbers were determined by the method proposed in A. S. T. M. Proc. 38, I 392 (1938). The specifications of fuel A and fuel B, together with the cetane number determinations on blends of these fuels containing representative addition agents of the type contemplated herein are set forth below.

Fuel A was a straight run number 2 fuel oil possessing the following characteristics:

|                                   |       |    |  |
|-----------------------------------|-------|----|--|
| Gravity, ° A. P. I.               | 39.8  |    |  |
| Flash point (Pensky-Martens, °F.) | 172   | 30 |  |
| Aniline point, °F.                | 160.5 |    |  |
| A. S. T. M. distillation:         |       |    |  |
| Initial °F.                       | 386   |    |  |
| 10%                               | 435   |    |  |
| 90%                               | 572   | 35 |  |
| End point                         | 614   |    |  |
| Diesel index                      | 63.9  |    |  |
| Cetane number                     | 56.5  |    |  |

#### Cetane number determinations

| Substance blended with fuel A      | Percent by weight added | Cetane number of blend | Increase in cetane number |
|------------------------------------|-------------------------|------------------------|---------------------------|
| p-Nitro benzene diazo methyl ether | 0.33                    | 61.5                   | 5.0                       |
| p-Nitro benzene diazo ethyl ether  | 0.5                     | 64.5                   | 8.0                       |

Fuel B was a catalytically cracked fuel oil prepared from Mirando gas oil and possesses the following characteristics:

|                                   |       |    |  |
|-----------------------------------|-------|----|--|
| Gravity, ° A. P. I.               | 26.8  |    |  |
| Flash point (Pensky-Martens, °F.) | 176   |    |  |
| Aniline point, °F.                | 101.2 |    |  |
| A. S. T. M. distillation:         |       |    |  |
| Initial °F.                       | 388   |    |  |
| 10%                               | 433   |    |  |
| 90%                               | 555   |    |  |
| End point                         | 630   |    |  |
| Diesel index                      | 27.1  |    |  |
| Cetane number                     | 21.7  | 60 |  |

#### Cetane number determinations

| Substance blended with fuel B      | Percent by weight added | Cetane number of blend | Increase in cetane number |
|------------------------------------|-------------------------|------------------------|---------------------------|
| p-Nitro benzene diazo methyl ether | 0.7                     | 27.2                   | 5.5                       |

It will be seen from the foregoing tabulations that the aromatic diazo alkyl ethers contemplated herein are effective to improve the ignition quality of Diesel fuels when added thereto in minor proportions. The amount of the compound used may be varied, depending upon the base fuel stock, etc., but in general it appears that amounts ranging from about 0.1 per cent to about 5.0 per cent will effect the desired improvement.

It is to be understood that the term Diesel fuel as used herein has reference to any hydrocarbon fuel adapted for use in an engine operating according to the Diesel cycle; also that the invention is not limited to the specific compounds or illustrative procedures described herein but that it includes within its scope such variations or modifications as fairly come within the spirit of the appended claims.

I claim:

1. An improved Diesel fuel having in admixture therewith a minor proportion of an aromatic diazo alkyl ether in sufficient amount to improve the ignition quality of the fuel.

2. An improved Diesel fuel having in admixture therewith a minor proportion of an aromatic diazo alkyl ether having a nitro substituent in the aromatic nucleus, the said compound being present in the fuel in an amount sufficient to improve the ignition quality thereof.

3. An improved Diesel fuel having in admixture therewith a minor proportion of a benzene diazo alkyl ether in an amount sufficient to improve the ignition quality of the fuel.

4. An improved Diesel fuel having in admixture therewith a minor proportion of a para-nitro benzene diazo alkyl ether in an amount sufficient to improve the ignition quality of the fuel.

5. An improved Diesel fuel having in admixture therewith a minor proportion of para-nitro benzene diazo methyl ether in an amount sufficient to improve the ignition quality of the fuel.

6. An improved Diesel fuel having in admixture therewith a minor proportion of para-nitro benzene diazo ethyl ether in an amount sufficient to improve the ignition quality of the fuel.

EDWIN M. NYGAARD.